

Patented July 14, 1925.

1,545,836

# UNITED STATES PATENT OFFICE.

WINTHROP STANLEY LAWRENCE, OF BROOKLYN, NEW YORK, AND FREDERICK W. BARKER, JR., OF MORRISTOWN, NEW JERSEY, ASSIGNEES TO KAUMAGRAPH CO., OF NEW YORK, N. Y., A CORPORATION OF NEW YORK.

## TRANSFER INK FOR MARKING LEATHER.

No Drawing.

Application filed April 7, 1923. Serial No. 630,641.

To all whom it may concern:

Be it known that we, WINTHROP STANLEY LAWRENCE and FREDERICK W. BARKER, Jr., citizens of the United States, residing at 55

5 Hanson Place, Brooklyn, in the city of New York, county of Kings, State of New York, and 41 Franklin Street, city of Morristown, county of Morris, State of New Jersey, have invented certain new and useful Improvements 10 in Transfer Ink for Marking Leather, of which the following is a specification.

This invention relates to a new and improved transfer ink.

One of the objects of this invention is to 15 provide a new and improved transfer ink for marking leather, rubber and some textiles.

Another object of this invention is to provide a new and improved transfer ink which 20 will not smear on the leather, which is less porous than textiles, and which will give a firm and non-smeary permanent impression on the leather in spite of the presence of the stuffing greases in said leather.

25 It has been discovered that a mixture of Venice turpentine and shellac produces a composition which is not attacked by the stuffing greases in leather. Shellac and butyl tartrate give a composition, whose 30 range of melting is so great that good results can be secured on hard, impervious leather surfaces, such as horse hide and roller lamb and the like. The composition of the above mentioned substances produces 35 a product which is very resistant to the greases and can be applied very efficiently. Since the cost of Venice turpentine is rather high, a substitute therefor can be made by combining rosin and butyl tartrate. A suitable 40 formula can be made up as follows:

Orange shellac in the flake form—12 parts by weight.

Pine rosin W. W.—12 parts.

Butyl tartrate— $2\frac{1}{2}$  parts.

45 The shellac is present in sufficient quantity to give the ink the desired qualities. For best results the shellac should comprise more than 33 $\frac{1}{3}$  percent by weight of the ink.

This formula can be slightly modified to 50 meet weather requirements by making it softer or harder.

The rosin should be free from dirt and grit and of the water-white quality.

Other esters could be substituted for butyl

tartrate but most of them are much more 55 expensive and in addition, most of them are more volatile than butyl tartrate which is a disadvantage.

It is not believed that any chemical reactions take place in mixing the above ingredients, which is done under suitable temperature conditions to secure a thorough mixture, but on exposure to the air some oxidation takes place on the surface of the ink. 60

The shellac is used for its working qualities and because it produces an ink which can be advantageously applied. Its principal utility is due to the fact that it is insoluble in oils and the like which are used 70 in the greases employed for stuffing leather. The rosin employed in the above formula is used as a diluent to lower the price and in addition it softens the ink and increases 75 the fluidity.

The butyl tartrate in combination makes the composition very elastic so that the ink does not flake off or crack when the leather is bent and it also softens the composition and lowers the melting point thereof. 80

The solid fusible ink produced according to the above formula is placed upon a paper back or base in the ordinary manner and is applied to the leather by means of a hot flat iron or the like in the ordinary manner. 85

Inks made according to this formula are used for marking both natural and artificial leather and also for marking rubber.

Another suitable formula could be made by combining one part by weight of shellac and a part of true Venice turpentine. This true Venice turpentine is an exudation from a foreign larch and has about the consistency of thick molasses. The shellac is used for the reasons before mentioned and the Venice turpentine is used as a softening agent. 90

The second mentioned formula is not as desirable as the first as it is not as useful for marking hard leathers.

The compositions before mentioned are made by first heating the proper amount of rosin until it begins to bubble and then stirring in the shellac as rapidly as possible while keeping the substance fluid at all times. 100

After the shellac is added and the mixture is homogeneous, the butyl tartrate is stirred in and then the bronze or pigment is also stirred in. When this is completed, 105

the composition is panned and kept in the solid state until ready for use. The composition can be kept hot for a couple of hours, if necessary.

5 In making the ink from Venice turpentine and shellac alone, the shellac is first melted and the Venice turpentine is added.

We have described preferred embodiments of our invention but it is clear that changes 10 and omissions could be made without departing from its spirit and whenever we refer to any substance or substances in the claims it is to be understood that such reference includes all substances equivalent thereto.

15 We claim:

1. A solid, fusible, non-smeary, adherent ink for marking leather and the like, said ink containing coloring matter, and also containing solid shellac in sufficient proportion 20 to render the ink resistant to greases said ink being free from any shellac solvent.

2. A solid, fusible, non-smeary, adherent ink for marking leather and the like, said ink containing coloring matter, solid shellac 25 in sufficient proportion to render said ink resistant to greases, and also containing a solid substance having a melting point lower than shellac and miscible with molten shellac said ink being free from any shellac solvent.

30 3. A solid, fusible, adherent, non-smeary ink for marking leather and the like, containing coloring matter, shellac, rosin, and an ester whose volatility is equal to or less than that of butyl tartrate, said ink containing a sufficient proportion of shellac to render it resistant to greases, the said rosin and ester being present in sufficient proportion to make the fused ink sufficiently fluid 35 to be taken up by the object to be marked.

4. A solid, fusible, adherent, non-smeary 40 ink for marking leather and the like, containing coloring matter, shellac, rosin and butyl tartrate, said ink containing a sufficient proportion of shellac to render it resistant to greases, and containing a sufficient proportion of rosin and butyl tartrate to render the fused ink sufficiently fluid to be taken up by the object to be marked.

45 5. A solid, fusible, non-smeary, adherent ink for marking leather and the like, containing 50 coloring matter embodied in a solid base which is resistant to the greasy stuffing ingredients found in leather said ink being free from any solvent for said base.

55 6. An ink according to claim 5 which contains shellac and other ingredients which render the melting temperature of the ink lower than that of shellac.

60 7. A solid, fusible, non-smeary, adherent ink consisting substantially of coloring matter, twelve parts by weight of shellac, twelve parts by weight of pine rosin, and two and a half parts by weight of butyl tartrate.

65 8. A method of making a solid, fusible, non-smeary, adherent ink for marking leather and the like, which consists in melting and heating rosin until it begins to bubble, then adding shellac while keeping the melt fluid and stirring the ingredients to produce a homogeneous mixture then adding an ester whose melting point is less than butyl tartrate, and stirring until the mixture is homogeneous and then adding the 70 pigment.

75 In testimony whereof we hereunto affix our signatures.

WINTHROP STANLEY LAWRENCE.  
FREDERICK W. BARKER, JR.